

**PROCESS FOR THE STABILIZATION OF CHLORINATED HYDROCARBONS**

Nestor Daras, Ixelles-Brussels, Belgium, assignor to Solvay & Cie., Brussels, Belgium, a Belgian company

No Drawing. Filed Dec. 9, 1958, Ser. No. 779,077

Claims priority, application Belgium Dec. 19, 1957

6 Claims. (Cl. 260—652.5)

The present invention relates to a process for the stabilisation of chlorinated hydrocarbons, particularly trichlorethylene and perchlorethylene, with a view of preventing the decomposition of these products and the simultaneous formation of acid during storage or in use.

It is known that by the action of heat and oxygen, chlorinated hydrocarbons undergo an oxidation which is catalysed by various agents such as light and certain metal salts, particularly iron, aluminium and magnesium salts.

In order to slow down this oxidation, it has been proposed to add to these chlorinated hydrocarbons small quantities of various products such as alcohols, mineral and organic basic products, phenols, epoxy compounds etc.

However effective these stabilisers may be for preventing the oxidation of chlorinated hydrocarbons, they are, in general incapable of preventing a rapid decomposition of these chlorinated hydrocarbons in the course of their use for the de-greasing of light metals, especially aluminium and its alloys.

The addition of one stabilising compound alone is in general, insufficient for preventing the decompositions of chlorinated hydrocarbons, particularly if they are used for the de-greasing of metals.

Moreover, the addition of several stabilising compounds does not always lead to the desired result, either because of their incompatibility, or because of the fact that too large quantities of products are necessary to ensure a good stabilisation.

It has already been proposed to combine the stabilising action of epoxy compounds such as epichlorhydrin with that of amines. A synergistic action would thus permit to reduce considerably the quantity of amines necessary for a good stabilisation, but when the chlorinated hydrocarbons are used for the de-greasing of light metals, the combined action of epichlorhydrin and certain amines such as triethylamine, cyclohexylamine, methoxypropylamine, dimethoxypropylamine, piperidine and aniline has proved, according to the test described below, to be inferior to that of epichlorhydrin alone.

It has also been proposed (U.S. patent application No. 771,754) to combine the stabilising action of epichlorhydrin with that of phenols, but important synergistic effects have hitherto been obtained only with phenol.

The present invention relates to a new combination of stabilising reagents leading to particularly valuable results.

According to the invention, chlorinated hydrocarbons, particularly trichlorethylene and perchlorethylene, are stabilised by adding small quantities of an alcohol and of a phenol.

All phenols the physical properties of which are compatible with the normal use of chlorinated hydrocarbons may be employed according to the process of the inven-

tion. Good results have been obtained particularly with phenol, cresols and thymol.

All alcohols the boiling point of which is near that of the hydrocarbon to be stabilised, may be used.

5 The action of phenols is combined, for example, with that of saturated or unsaturated aliphatic alcohols such as tertiary or normal butyl alcohol, tertiary amyl alcohol, ethylenic or acetylenic alcohols such as allyl alcohol, methylbutynol, diol ethers such as methylcellosolve or 10 monomethyl ether of ethylene glycol and the like.

The stabilising action of the various compounds used for improving the resistance to decomposition of chlorinated hydrocarbons is demonstrated by an accelerated laboratory test which is carried out as follows:

15 150 cc. of, for example, trichlorethylene and a test piece of aluminium are placed in a 300 cc. flask of a Soxhlet extracting apparatus fitted with a 65 cc. extractor. The flask is electrically heated and the trichlorethylene is rapidly brought to the boil under reflux at a constant

20 rate, while an oxygen stream is passed through the apparatus which is illuminated by a fluorescent lamp of the "Blue actinic" type. During the whole duration of the test, the rate of evolution of acid vapours at the outlet of the apparatus is measured. This rate which is very 25 low at the start becomes suddenly very high, whilst the trichlorethylene turns black and is transformed into a black tarry mass.

The resistance of trichlorethylene to the test is measured by time, expressed in hours, counted from the start of the test, i.e. as soon as the sample is brought to

30 the boil, to the instant where the evolution of acid suddenly becomes very rapid and exceeds  $15 \cdot 10^{-3}$  mol. g./h. The following Table 1 shows the resistance to decomposition of unstabilised trichlorethylene and of trichlorethylene 35 stabilised with various phenol compounds and/or alcohols.

Table 1

| 40 | Test No.                                      | Stabilizing substances, mg./l. | Resistance in the accelerated test, hrs. |
|----|-----------------------------------------------|--------------------------------|------------------------------------------|
| 1  | Nil                                           |                                | 22                                       |
| 2  | normal butyl alcohol (1,500)                  |                                | 23                                       |
| 3  | tertiary butyl alcohol (1,500)                |                                | 37                                       |
| 4  | tertiary amyl alcohol (1,500)                 |                                | 33                                       |
| 5  | methylcellosolve (1,500)                      |                                | 35                                       |
| 6  | allyl alcohol (1,500)                         |                                | 58                                       |
| 7  | methylbutynol (1,500)                         |                                | 40                                       |
| 8  | phenol (100)                                  |                                | 64                                       |
| 9  | phenol (200)                                  |                                | 95                                       |
| 10 | o. cresol (200)                               |                                | 130                                      |
| 11 | thymol (100)                                  |                                | 35                                       |
| 12 | phenol (100)—normal butyl alcohol (1,500)     |                                | 122                                      |
| 13 | phenol (100)—tertiary butyl alcohol (1,500)   |                                | 137                                      |
| 14 | phenol (100)—tertiary amyl alcohol (1,500)    |                                | 155                                      |
| 15 | phenol (200)—tertiary amyl alcohol (1,500)    |                                | 280                                      |
| 16 | o. cresol (200)—tertiary amyl alcohol (1,500) |                                | 390                                      |
| 17 | thymol (100)—tertiary amyl alcohol (1,500)    |                                | 92                                       |
| 18 | phenol (100)—allyl alcohol (1,500)            |                                | 135                                      |
| 19 | phenol (100)—methylcellosolve (1,500)         |                                | 147                                      |
| 20 | phenol (100)—methylbutynol (1,500)            |                                | 144                                      |
| 21 | phenol (200)—methylbutynol (1,500)            |                                | 220                                      |

60 The tests 12 to 21 show that by combining the stabilising action of phenols with that of alcohols, there is obtained a resistance of chlorinated hydrocarbons to decomposition which is superior to the sum of results obtainable by using the compounds separately.

The synergistic effect is particularly marked when 65 tertiary alcohols are combined with phenols.

This effect increases with the phenol content, but it is already very substantial at phenol concentrations of 100 to 200 mg./litre.

It is possible to add to the combination of substances 70 which form the object of the invention, other compounds known for their stabilising action. The resistance to decomposition is particularly increased by adding pyrrole,

pyrrole derivatives or aniline, as can be seen from the tests listed in the following Table 2.

Table 2

| Test No. | Stabilizing substances, mg./l.                           | Resistance in accelerated test, hrs. |
|----------|----------------------------------------------------------|--------------------------------------|
| 22       | pyrrole (100)                                            | 84                                   |
| 23       | pyrrole (200)                                            | 164                                  |
| 24       | pyrrole (100)+phenol (100)                               | 158                                  |
| 25       | phenol (100)+tertiary amyl alcohol (1,500)+pyrrole (100) | 269                                  |
| 26       | phenol (200)+tertiary amyl alcohol (1,500)+pyrrole (200) | >500                                 |
| 27       | tertiary amyl alcohol (1,500)+pyrrole (200)              | 206                                  |
| 28       | aniline (200)                                            | 22                                   |
| 29       | phenol (100)+aniline (100)                               | 82                                   |
| 30       | tertiary amyl alcohol (1,500)+aniline (200)              | 53                                   |
| 31       | phenol (100)+tertiary amyl alcohol (1,500)+aniline (100) | 201                                  |
| 32       | phenol (200)+tertiary amyl alcohol (1,500)+aniline (200) | >500                                 |

Compared with the tests 14—13 of Table 1, the tests 25—26 and 31—32 show that pyrrole and aniline are advantageously combined with binary alcohol-phenol stabilisers and noticeably increase the synergistic effect. In contrast to this, the same compounds combined with an alcohol alone or a phenol alone lead only to additive results.

The resistances of more than 500 hours which have been found are extraordinary when taking into account that during the accelerated test the boiling chlorinated hydrocarbon is simultaneously subjected to the action of oxygen and light in the presence of aluminium.

The quantities of stabilising matters to be used according to the process of the invention may generally be comprised between 0.05 and 0.5 g./litre of phenol and between 0.5 to 10 g./litre of alcohol. The most advantageous proportions seem to be 0.1 to 0.25 g. of phenol and 1 to 3 g. of alcohol per litre of hydrocarbon to be stabilised.

Small quantities of pyrrole derivatives and/or of aniline appreciably increase the resistance of chlorinated hydrocarbon to decomposition. The latter compounds are advantageously added at a ratio of 0.05 to 0.5 g./litre, but considerably smaller proportions are already effective.

Although the stabilising compounds based on phenols and/or alcohols are particularly effective in the stabilisation of trichlorethylene, one of the chlorinated hydrocarbons which are most sensitive to decomposition, they may also be used for the stabilisation of perchlorethylene

and of other chlorinated solvents such as carbon tetrachloride, dichlorethane, trichlorethane and the like.

I claim:

1. A process for the stabilization of a chlorinated hydrocarbon solvent to inhibit its decomposition and the simultaneous formation of acids, which comprises adding to said solvent 0.05 to 0.5 g. of a phenol selected from the group consisting of phenol and the cresols, and 0.5 to 10 g. of tertiary amyl alcohol per liter of said chlorinated hydrocarbon solvent.
2. A process for the stabilization of a chlorinated hydrocarbon solvent to inhibit its decomposition and the simultaneous formation of acids, which comprises adding to said solvent 0.05 to 0.5 g. of a phenol selected from the group consisting of phenol and the cresols, 0.5 to 10 g. of a tertiary amyl alcohol, and 0.05 to 0.5 g. of a compound selected from the group consisting of pyrrole and aniline per liter of said chlorinated hydrocarbon solvent.
3. A process for the stabilization of trichlorethylene to inhibit its decomposition and the simultaneous formation of acids, which comprises adding to said trichlorethylene 0.05 to 0.5 g. of a phenol selected from the group consisting of phenol and the cresols, and 0.5 to 10 g. of tertiary amyl alcohol per liter of said trichlorethylene.
4. A composition of matter comprising a chlorinated hydrocarbon solvent, 0.05 to 0.5 g. of a phenol selected from the group consisting of phenol and the cresols, and 0.5 to 10 g. of tertiary amyl alcohol per liter of said chlorinated hydrocarbon solvent.
5. A composition of matter comprising trichlorethylene, 0.05 to 0.5 g. of a phenol selected from the group consisting of phenol and the cresols, and 0.5 to 10 g. of tertiary amyl alcohol per liter of said trichlorethylene.
6. A composition of matter comprising trichlorethylene, 0.05 to 0.5 g. of a phenol selected from the group consisting of phenol and the cresols, 0.5 to 10 g. of tertiary amyl alcohol, and 0.05 to 0.5 g. of a compound selected from the group consisting of pyrrole and aniline per liter of said trichlorethylene.

#### References Cited in the file of this patent

#### UNITED STATES PATENTS

- |           |                       |               |
|-----------|-----------------------|---------------|
| 2,371,644 | Petering et al. ----- | Mar. 20, 1945 |
| 2,797,250 | Copelin -----         | June 25, 1957 |
| 2,803,676 | Willis et al. -----   | Aug. 20, 1957 |
| 2,911,449 | Herman et al. -----   | Nov. 3, 1959  |

#### FOREIGN PATENTS

- |         |                     |               |
|---------|---------------------|---------------|
| 787,726 | Great Britain ----- | Dec. 11, 1957 |
|---------|---------------------|---------------|